

## UNITED STATES PATENT OFFICE

2,260,304

## SYNTHETIC OIL ADDITION AGENTS

Ernest F. Engelke, Merchantville, N. J., assignor  
to Cities Service Oil Company, New York, N. Y.,  
a corporation of Pennsylvania

No Drawing. Application September 15, 1939,  
Serial No. 295,037

## 11 Claims.

(Cl. 252—48)

This invention relates to oil products containing and improved by the presence therein of certain organic halogenated phosphine compounds.

Organic phosphine compounds have been added to lubricating oils and other preparations for various purposes, as for example, Butz has proposed the use of phosphine oxides and sulfides in his Patent No. 2,138,835, as addition agents for lubricating stocks. These were proposed particularly for increasing the extreme pressure characteristics of the oil stocks.

A number of investigators have also found that certain phosphorus compounds successfully inhibit the corrosion of certain of the bearing alloys used in automobile engines. Such bearings as cadmium-silver, cadmium-nickel and copper-lead have been found to be more or less readily corroded by the usual motor oils, particularly those oils made by solvent extraction processes. Addition agents which inhibit corrosion therefore are of considerable advantage, not only because they prevent or reduce corrosion of motor bearings, but because they tend to prevent deterioration of the motor oils from the catalytic effects of the metals with which they come in contact.

The primary object therefore of the present invention is to provide new and useful organic halogen-containing phosphine compounds which will improve motor oils and other lubricants, prevent deterioration of the oil and inhibit corrosion of the motor bearings.

A further object of the invention is to provide organic halogenated phosphine addition agents which can be used in relatively small proportions in lubricants and other products to improve their life and utility.

Accordingly, the present invention contemplates improved halogenated phosphine compounds for use as addition agents, comprising particularly organic halogenated phosphine oxides or sulfides in which the halogen is directly attached to phosphorus. The preferred compounds preferably contain no nitrogen because phosphine-nitrogen derivatives such as amino compounds are as a rule very difficult to dissolve in mineral oils, or to be held in solution once they have been dissolved under favorable conditions, such as at much higher temperatures than are employed in their use. The halogenated phosphine compounds of the present invention contain at least one organic radical such as an alkyl, aryl, aralkyl, hydroaryl or a heterocyclic radical. Such radicals may be directly attached to the phosphorus through a carbon atom but are preferably at-

tached through an oxygen or sulfur atom as in the case of alcohols, phenols, mercaptans and thiophenols. The preferred compounds furthermore contain at least one halogen atom, directly attached to phosphorus, and an oxygen or a sulfur atom, also directly attached to phosphorus (by a double bond).

The method of making the improved addition agents of the present invention may be illustrated by describing the steps used in the making of a di-cresol chlorophosphine sulfide. One mol of phosphorus tri-chloride is reacted with two mols of a cresol (or mixture of cresols) at ordinary room temperature until the evolution of hydrochloric acid gas substantially ceases, after which the mixture is heated on a steam bath to complete the reaction. The resulting product is a di-cresol mono-chlorophosphine which is purified by distillation at a low pressure of from 1 to 2 mm. of Hg. A satisfactory purification however consists in topping off the light material to a temperature of about 400° F. at 11 mm. of Hg. The sulfide may be readily produced by reacting the di-cresol mono-chlorophosphine with one equivalent of sulfur at a temperature of from 360° to 380° F. The resulting product is a di-cresol mono-chlorophosphine sulfide. The phosphine oxide may be produced by treating the di-cresol mono-chlorophosphine with hydrogen peroxide or nitric acid to oxidize the phosphine to the phosphine oxide. The di-chlorophosphine derivatives may be made by reacting one mol of phosphorus trichloride with one mol of the desired organic compound such as a phenol or a thiophenol.

The phosphine sulfide produced by the above procedure may be purified by digestion with strong caustic soda and thereafter washing it with water, whereupon the product when recrystallized from alcohol has a melting point of from 120° to 130° F. When the products are made from mixed organic compounds such as mixed phenols or cresols, they have a very indefinite melting point and tend to remain in liquid state at temperatures considerably below their normal melting points. Both the mono- and di-chlorophosphines have been found to be very stable compounds, not saponifiable by boiling with water, alkalis or concentrated hydrochloric acid. The organic mono-chlorophosphine derivatives are soluble in alcohol ether and chloroform, and considerably more soluble in the coastal type oils than in the heavy paraffinic Pennsylvania type oil stocks, but even the latter readily dissolve more than is necessary.

The improved addition agents of the present invention may be used alone as a film strength agent or mixed with any grade of lubricating oil, liquid hydrocarbon, mineral oil or oily or grease compositions. The organic radicals or groups in any one of the halogenated phosphine derivatives may be alike or different, and one or more such groups may contain separate halogen atoms. The presence of chlorine or other halogen atoms such as fluorine, bromine and iodine, has been found to effectively increase the film strength characteristics of such compounds. Each of the organic groups or radicals also preferably contains at least six carbon atoms, although such radicals containing less than six atoms of carbon in certain cases possess merit.

Examples of specific compounds used as addition agents in accordance with the present invention are:

Di-phenol-O-mono-chlorophosphine oxide  
Di-cresol-O-mono-chlorophosphine oxide  
Di-butyl mono-chlorophosphine oxide  
Di-amyl mono-chlorophosphine oxide  
Di-benzyl mono-chlorophosphine oxide  
Mono-phenol-O-di-chlorophosphine oxide  
Mono-cresol-O-di-chlorophosphine oxide  
Mono-butyl di-chlorophosphine oxide  
Mono-benzyl di-chlorophosphine oxide  
Di-phenol-O-mono-chlorophosphine sulfide  
Di-ortho, meta and para cresol-O-mono-chlorophosphine sulfide  
Di-butyl mono-chlorophosphine sulfide  
Di-benzyl mono-chlorophosphine sulfide  
Di-thiophenol-S-mono-chlorophosphine sulfide  
Di-ortho, meta and para thiocresol-S-mono-chlorophosphine sulfide  
Di-thiobutyl-S-mono-chlorophosphine sulfide  
Di-thiobenzyl-S-mono-chlorophosphine sulfide  
Di-thienyl-S-mono-chlorophosphine sulfide  
Di-thiophenol-S-mono-chlorophosphine oxide  
Di-ortho, meta and para thiocresol-S-mono-chlorophosphine oxide  
Di-thiobutyl-S-mono-chlorophosphine oxide  
Di-thiobenzyl-S-mono-chlorophosphine oxide  
Di-thienyl-S-mono-chlorophosphine oxide  
Di-hydroxybutyl-O-mono-chlorophosphine oxide  
Di-hydroxybutyl-O-mono-chlorophosphine sulfide  
Mono-hydroxybutyl-O-di-bromophosphine oxide  
Mono-hydroxybutyl-O-di-bromophosphine sulfide

The -S- and -O- symbols used in the foregoing list of compounds indicate the fact that the organic groups are attached to phosphorus through the oxygen and sulfur atoms in the organic group.

The compounds of the present invention are effective for preventing or inhibiting the corrosion of various bearing metals such as those used in automobile motors. This effectiveness may be illustrated by comparison of the results of tests made on certain bearing metals with a Pennsylvania lubricating oil of S. A. E. 20, and this same oil containing an added compound. The oil alone showed substantial corrosion of bronze-babbitt and cadmium-copper-silver alloys, but from 1% to 1.5% of di-phenol-O-mono-chlorophosphine oxide and of di-paracresol-O-mono-chlorophosphine sulfide in the oil substantially inhibited corrosion in each instance.

Tests were also carried out to determine the effect of the halogenated phosphine compounds of the present invention in decreasing engine bearing wear with respect to various types of

bearing alloys. Tests were conducted on the alloys: cadmium - copper - silver, copper - lead, bronze-babbitt and babbitt, all of which were very substantially worn by the use of a 20 S. A. E. solvent treated oil which contained no addition agent. The same was true with a Pennsylvania 20 S. A. E. oil not produced by solvent extraction, although the corrosion for babbitt was somewhat less. The wear was very greatly decreased with both types of oil containing 0.5% of di-cresol-O-mono-chlorophosphine sulfide.

Further tests were also made to determine the film strength of the oil alone and the oil containing addition agents prepared in accordance with the present invention. The 20 S. A. E. Pennsylvania motor oil alone had a load carrying capacity on the Timken testing machine of 8700 lbs. per square inch with the machine operated at 500 R. P. M. and a rubbing speed of 250 feet per minute, at a temperature of 150° F. Comparative tests on the same oil containing 0.5%, 1.0% and 1.5% of di-phenol-O-mono-chlorophosphine sulfide showed load-carrying capacities respectively of 11,000, 14,400 and 18,300 lbs. per square inch. These same proportions of di-paracresol - O - mono-chlorophosphine sulfide showed load carrying capacities respectively of 14,200, 18,000 and 19,200 lbs. per square inch.

While the foregoing examples illustrating the properties and applications of the improved compounds relate primarily to their use in mineral oils, it is to be understood that the invention includes their use as such or in any mixtures for all purposes to which they are adapted. A mixture of two or more compounds may be used as an addition agent. For example, they have been found useful in cutting oils and in lubricants for the bearings and cylinder wall surfaces of internal combustion engines. The compounds may also be used as anti-rust agents, film strength agents in greases, and in blends containing fatty oils, synthetic oils and esters, or they may be used alone as film strength agents for any desired use where the maintenance of a surface film between moving parts of a mechanism is essential.

The improved compounds of the present invention have been found particularly useful in the crank case of an automobile, since in a lubricant vehicle they maintain a relatively clear oil over substantially long periods of use. The compounds are also effective ingredients of crank case flushing compositions because they aid in dissolving resinous constituents in the motor and crank case and at the same time provide an effective lubricant in light oil solvents or mixtures. Flushing oils therefore containing such compounds may be used in a motor operated for substantial periods of time while the crank case is being cleaned and flushed. A suitable flushing mixture may contain from 1% to 5% of one or more of the compounds, dissolved in relatively large proportions of light oils such as kerosene, light furnace oil, light coal tar distillates or mixtures of these oils.

The phosphine compounds of the present invention may be used as top cylinder lubricants in internal combustion engines by adding approximately 1% by volume thereof to the motor fuel to be used in the engine. The improved phosphine compounds may also be employed for other purposes as will be apparent to those skilled in the art.

Having thus described the invention in its preferred form, what is claimed as new is:

1. A composition of matter comprising a lubricating oil containing a relatively small proportion of a nitrogen-free organic chlorophosphine oxide in which chlorine is directly attached to phosphorus.
2. A composition of matter comprising a hydrocarbon oil containing approximately 1% of a nitrogen-free organic chlorophosphine oxide in which chlorine is directly attached to phosphorus.
3. A composition of matter comprising a hydrocarbon oil and a relatively small proportion of a nitrogen-free di-cresol-O-mono-chlorophosphine oxide in which the chlorine is directly attached to phosphorus.
4. A composition of matter comprising a hydrocarbon oil containing a relatively small proportion of a cresol-O-chlorophosphine sulfide in which chlorine is directly attached to phosphorus.
5. A composition of matter comprising a hydrocarbon oil and a relatively small proportion of an organic halogenated phosphine oxide in which the halogen is directly attached to phosphorus and in which each organic radical contains at least six carbon atoms.
6. A lubricant comprising a hydrocarbon oil and a halogenated phosphine oxide in which a halogen is directly attached to phosphorus and which contains an organic radical directly attached to phosphorus and selected from the group consisting of alkyl, aryl, hydroxyalkyl, haloalkyl, haloaryl, hydroxyaryl, phenolic, mercapto, thiophenoilic, aralkyl, hydroaryl and heterocyclic groups.
7. A lubricant comprising a hydrocarbon oil and a relatively small proportion of a compound selected from the group consisting of nitrogen-free organic halogenated phosphine oxides and sulfides in which halogen is directly attached to phosphorus.
8. A composition of matter comprising a hydrocarbon oil containing a relatively small proportion of a nitrogen-free di-cresol-O-chlorophosphine sulfide in which chlorine is directly attached to phosphorus.
9. A composition of matter comprising a hydrocarbon oil containing a relatively small proportion of a di-thio-phenol-S-chlorophosphine oxide in which chlorine is directly attached to phosphorus.
10. A composition of matter comprising a hydrocarbon oil and a small proportion of a compound selected from the group consisting of nitrogen-free organic halogenated phosphine oxides and phosphine sulfides in which halogen is directly attached to phosphorus.
11. A composition of matter comprising a hydrocarbon oil and a relatively small proportion of a nitrogen-free compound selected from the group consisting of organic halogenated phosphine oxides and phosphine sulfides and mixtures thereof in which halogen is directly attached to phosphorus, and wherein each organic radical in the compound consists of a radical containing at least six carbon atoms and selected from the group consisting of alkyl, aryl, aralkyl, hydroaryl, heterocyclic, hydroxyalkyl, hydroxyaryl, phenolic, mercapto, thiophenoilic, haloalkyl and haloaryl radicals.

35

ERNEST F. ENGELKE.